

## UNITED STATES PATENT OFFICE

ROBERT S. ARCHER, OF LAKEWOOD, AND LOUIS W. KEMPF, OF CLEVELAND, OHIO, AS  
SIGNORS TO ALUMINUM COMPANY OF AMERICA, OF PITTSBURGH, PENNSYLVANIA,  
A CORPORATION OF PENNSYLVANIA

## ALUMINUM-SILICON ALLOYS

No Drawing. Application filed December 23, 1930. Serial No. 504,422.

This invention relates to aluminum base alloys containing silicon, and has for an important object to provide alloys in which the elongation is markedly improved over that heretofore obtainable with the same class of alloys.

A further object of the invention is the provision of aluminum base alloys containing silicon in which other physical properties such as tensile strength are satisfactorily commensurate with the improved elongation.

A still further object of the invention is the provision of a series of aluminum base alloys containing silicon in which the elongation can be suitably varied to a predetermined extent by a proper choice of the alloying constituents.

Another object of the invention is the provision of aluminum base alloys containing silicon which in cast or other fabricated form can be used under conditions subjecting the article to elevated temperatures and will at such temperatures retain a high proportion of the strength and hardness exhibited at ordinary temperatures.

The aluminum base alloys containing silicon are characterized by low specific gravity which has made them both useful and desirable for many purposes. When applied to certain uses which give rise to exacting requirements their strength and hardness have not at all times proved adequate, and it has been found that these properties may be considerably improved by the addition of small quantities of magnesium, as described in the copending application of L. W. Kempf, Serial No. 463,576. For many purposes these latter alloys with magnesium have proved quite satisfactory but at times it becomes desirable to simultaneously obtain in an alloy the low specific gravity and the strength and hardness of the aluminum-silicon-magnesium alloys with an elongation improved to an extent not heretofore attained in related cast alloys of this class.

One of the inherent disadvantages which have restricted the use of aluminum base alloys containing silicon, with or without other alloying ingredients, has been the difficulty in finding alloys of this nature with satisfactory elongation and which can be readily cast. As the amount of silicon is increased, say from about 2.5 per cent to about 14 per cent, the elongation decreases to a comparatively low figure. In adding even small amounts of magnesium to the ordinary aluminum-silicon alloys we have observed that although the strength and hardness are improved the elongation is not appreciably increased if at all. We have, however, discovered that if the amount of iron present as an impurity be controlled by restricting it to less than 0.4 per cent, a remarkable improvement is evidenced in the elongation not only without loss of strength but even with the strength increased. We have discovered in addition that small quantities of copper, up to about 1.50 per cent, will in the heat-treated condition materially increase both strength and elongation.

We have also found that alloys within the scope of our invention containing varying amounts of silicon and magnesium with or without the addition of small amounts of copper are amenable to marked improvement by heat treatments now well known in the art, consisting of, for example, heating the alloys at from about 500° C. to 575° C. for a number of hours, say from 2 to 20 hours, followed by quenching. This treatment is usually known as the "solution" treatment. Even after the alloys have been thus improved by heat-treatment it is observed that those alloys in which the iron content has been controlled as hereinbelow described show a material improvement in elongation and also usually in strength over the ordinary alloys of this nature in which no effort has been made to confine the iron content be-

low the customary amount usually present as an impurity in the final alloy.

The commercial grade of aluminum ingot which is generally used in compounding alloys may contain approximately 0.5 per cent iron and this will be increased if the molten aluminum has any extended contact with iron pots or labels. As evidence of this tendency standard specifications compiled by the American Society for Testing Materials call for an impurity range of 0.5 to 0.8 per cent in a widely used aluminum alloy containing 13.0 per cent silicon.

We have found that if a very good elongation is desired in an ordinary casting the silicon content should preferably be between 2.5 per cent and 6 per cent, small amounts of other ingredients such as magnesium and in some cases copper being added as required. Improved casting properties may be secured by making use of silicon contents between 6 per cent and 10 per cent. A series of widely used commercial alloys are found between 10 per cent silicon and about 14 per cent silicon, which offer good strength and elongation, particularly when modified by such methods as outlined in United States Patents Nos. 1,387,900, 1,410,461 or 1,572,459. In these separate classes of alloys it will be found that the elongation can be markedly increased by keeping the iron content less than 0.4 per cent.

Typical effects of decreasing iron content on the elongation and tensile strength of aluminum base alloys containing silicon and magnesium are given in Table A below, obtained with a series of alloys each member of which contained about 7.5 per cent silicon and 0.3 per cent magnesium, with the iron content varying as shown. Tensile specimens from these alloys were cast in sand, heat-treated for 20 hours at 538° C., and quenched in water, with the following results:

Table A

| Per cent iron content: | Tensile strength lbs. per sq. in. | Elongation in 2 in. |
|------------------------|-----------------------------------|---------------------|
| 0.4                    | 30,470                            | 3.7 per cent        |
| 0.2                    | 29,630                            | 4.8 per cent        |
| 0.15                   | 31,480                            | 7.1 per cent        |

It will be observed that when the iron content is lowered to 0.15 per cent the elongation is practically doubled and the tensile strength has increased slightly.

Table B below shows the effect of decreasing iron content on the elongation and tensile strength of aluminum base alloys containing 5 per cent silicon, 0.8 per cent magnesium and 0.25 per cent copper, the iron content varying as shown. Tensile specimens were cast

in sand, heat-treated for 20 hours at 538° C. and quenched in water.

Table B

| Per cent iron content | Tensile strength lbs. per sq. in. | Elongation in 2 in. |
|-----------------------|-----------------------------------|---------------------|
| 1.0                   | 28,060                            | 2.2 per cent        |
| 0.4                   | 27,060                            | 3.2 per cent        |
| 0.2                   | 30,260                            | 5.6 per cent        |
| 0.15                  | 31,630                            | 10.1 per cent       |

It is observed that there is a marked increase in elongation as the iron content is lowered and there is a substantial increase in tensile strength. Table C indicates the effect of a lower iron content on the tensile strength and elongation of aluminum base alloys containing 10 per cent silicon, 0.2 per cent magnesium and 0.1 per cent copper, the iron content varying as shown. Tensile specimens were cast in sand, given a solution treatment at 552° C. and quenched in water. Preceding the casting of the alloys they were modified with an alkaline reagent by a process familiar to those skilled in the art and outlined in one of the United States patents numbered hereinabove, which consists, briefly, in introducing into the molten alloy an alkaline reagent which refines the silicon constituent present in the alloy.

Table C

| Per cent iron content | Tensile strength lbs. per sq. in. | Elongation in 2 in. |
|-----------------------|-----------------------------------|---------------------|
| 0.69                  | 28,580                            | 10.2 per cent       |
| 0.47                  | 30,740                            | 14.0 per cent       |
| 0.14                  | 33,270                            | 18.7 per cent       |

It will be noted that although the elongation with the high iron content is very favorable (due to the modifying process), further improvement is obtained as the iron is decreased. Even though the elongation of the alloy decreases with increasing silicon the elongation can nevertheless be improved by the methods we outline. Although the alloys will show a distinct improvement on modification, especially in the higher silicon ranges, we have discovered that an additional marked improvement over the modified condition can be produced by restricting the iron content to less than about 0.4 per cent. The combination of properties illustrated in Table C above, exemplified by the alloy containing 0.14 per cent iron, is extremely desirable in view of the low specific gravity of alloys, their amenability to heat-treatment, and their potentialities for improvement by the modification process.

We have also found that in the heat treated condition the presence of appreciable quantities of copper effects a substantial improvement in certain of the physical properties,

for instance tensile strength, elongation, and hardness, and we have effected improvements over a range of about 2.5 to 14 per cent silicon and 0.1 per cent to 3 per cent magnesium (preferably not more than about 0.5 per cent) by varying the copper from about 0.1 per cent (preferably not more than about 1.5 per cent), even when the iron content is considerably more than 0.4 per cent. If very good elongation is desired in an ordinary casting the silicon content should preferably be between 2.5 and 6 per cent. Improved casting properties may be secured by making use of silicon contents between 6 per cent and 10 per cent. A series of widely used commercial alloys are found between 10 per cent and 14 per cent silicon, which offer good strength and elongation, particularly when modified by such methods as outlined in 20 United States Patents 1,387,900, 1,410,461, or 1,572,459.

Table D gives examples of the increase in strength, elongation and hardness effected by additions of copper, as shown by cast test specimens of an alloy containing about 7.0 per cent silicon, about 0.33 per cent magnesium and about 0.16 per cent iron with the copper varying as shown in Table D below. These specimens were heated for 20 hours at 538° C. and quenched.

Table D

| Per cent copper | Tensile strength lbs. per sq. in. | Elongation in 2 in. | Brinell hardness |
|-----------------|-----------------------------------|---------------------|------------------|
| 0.02            | 31,480                            | 7.1 per cent        | 63.5             |
| 0.77            | 33,770                            | 7.3 per cent        | 71.8             |
| 1.26            | 38,160                            | 7.4 per cent        | 80.2             |

40 In an alloy of lower silicon content a very marked increase in strength and elongation was obtained with an increase in copper. The alloy contained approximately 5.0 per cent silicon, 0.37 per cent magnesium and 0.16 per cent iron with copper as shown in Table E below. Sand cast specimens were heat treated for 20 hours at 538° C. and quenched.

Table E

| Per cent copper | Tensile strength lbs. per sq. in. | Elongation in 2 in. | Brinell hardness |
|-----------------|-----------------------------------|---------------------|------------------|
| 0.02            | 25,810                            | 5.0 per cent        | 58               |
| 0.25            | 31,530                            | 10.1 per cent       | 64               |

45 The elongation was more than doubled with an increase in copper from .02 to .25 per cent while the strength was increased more than 5,000 pounds per square inch and the Brinell hardness was increased from 58 to 64.

50 Table F shows the effect of decreasing iron

content on an aluminum base-alloy containing 5 per cent silicon, 0.3 per cent magnesium, and 0.75 per cent copper, the iron varying as shown. Tensile specimens were cast in sand, heated for 20 hours at 538° C., and quenched in water.

Table F

| Percent iron content | Tensile strength lbs. per sq. in. | Elongation in 2 in. |
|----------------------|-----------------------------------|---------------------|
| 1.0                  | 29,200                            | 2.5 per cent        |
| 0.4                  | 29,800                            | 3.3 per cent        |
| 0.2                  | 32,100                            | 4.8 per cent        |
| 0.15                 | 34,670                            | 8.9 per cent        |

75

80

85

90

95

100

105

110

115

120

125

130

15 A number of alloys were subjected to varying conditions of temperature to determine the effect on their physical properties, the results being largely influential in our choice 20 of the particular alloy to use where the product is exposed to temperature elevated beyond the ordinary. In one variety of test the alloys were given a solution treatment and subsequently reheated for a certain time at a lower temperature. Physical properties were determined both after the solution treatment and after the reheating treatment. Of all the alloys tested under the so-called "solution" and "stabilization" treatments the alloys containing copper suffered the least deterioration. Increasing the copper content was effective in decreasing the softening caused by the stabilization treatment.

25 As an example two alloys were chosen which contained approximately 0.4 per cent iron, 5.0 per cent silicon and 0.5 per cent magnesium. The variation in copper content is shown in Table G below. Sand cast bars from the alloys were heated for 18 hours at 550° C., quenched and reheated for 6 hours at 315° C. The result of tests after the solution treatment and also after the stabilization heat treatment are shown in the table.

Table G

|                                                              | Per cent Cu 0.14 | Per cent Cu 0.85 |
|--------------------------------------------------------------|------------------|------------------|
| Tensile strength lbs. per sq. in. after solution treatment   | 28,341           | 29,700           |
| Tensile strength lbs. per sq. in. after treatment at 315° C. | 22,700           | 27,650           |
| Loss in strength                                             | 5,633            | 2,050            |

30 Two significant facts may be noted from the table. One is that the increase in copper content effected an increase in tensile strength after the solution heat treatment. The other is that the secondary heat treatment had considerably less injurious effect on the alloy with the greater copper content.

35 In compounding the alloys it will be found advantageous to begin with aluminum ingot of high purity. It will be recognized that

iron may be picked up in the melting processes and that in order to assure a final iron content of less than 0.4 per cent it may be necessary to start with aluminum ingot of lower iron content than 0.4 per cent. Melting or holding pots may be of non-ferrous composition if necessary. The other constituents may be added to the molten aluminum in the customary manner, the silicon and copper, for instance, by means of "rich alloys" and the magnesium in the pure state, to give the desired amount of these constituents in the final alloy, having due regard to the copper content, if any, in the aluminum ingot and in scrap metal, or metal of previous melts, etc., that the foundry may desire to use up. However, our invention does not require a set technique in compounding the alloy since this can well be varied to suit foundry practice.

It is to be understood that in the appended claims the term "alloy" is used as including the alloy in the cast condition whether cast in sand or in any other type of mold, whether heat-treated or unheat-treated and whether modified or unmodified.

We claim:

1. A heat treatable alloy composed chiefly of aluminum and containing silicon between about 2.5 and 14 per cent, magnesium between about 0.1 and 0.5 per cent, and copper between about 0.1 and 1.5 per cent.
2. An aluminum base alloy containing from about 2.5 per cent to about 14 per cent silicon, from 0.1 per cent to 0.5 per cent magnesium, and from about 0.1 per cent to about 1.25 per cent copper, the iron content being less than about 0.4 per cent.
3. An aluminum base alloy containing from about 10 per cent to about 14 per cent silicon, from 0.1 per cent to about 0.5 per cent magnesium, and from about 0.1 per cent to about 1.25 per cent copper, the iron content being less than about 0.4 per cent.

45 In testimony whereof we hereto affix our signatures.

ROBERT S. ARCHER.  
LOUIS W. KEMPF.